

**1**

3,325,423

**UNIFIED CORROSION INHIBITOR**

Charles B. Jordan, Aberdeen, Md., assignor to the United States of America as represented by the Secretary of the Army  
No Drawing. Filed June 24, 1965, Ser. No. 466,866  
7 Claims. (Cl. 252—389)

The invention described herein may be manufactured and used by or for the Government for governmental purposes, without the payment to me of any royalty thereon.

This application is a continuation-in-part of application, Ser. No. 174,652, filed Feb. 20, 1962, for "Multipurpose Corrosion Inhibitor," now abandoned.

This invention relates to an improved corrosion inhibitor of the tetraborate type. More particularly, it relates to a novel tetraborate composition which provides improved corrosion inhibiting properties for organic fluids such as hydraulic brake fluids, antifreeze compounds, shock absorber fluids, polar recoil oils and the like.

Hydraulic fluids, antifreeze compounds and other related fluids are generally corrosive to metals found in the brake and cooling systems of vehicles. Due to the presence of a wide variety of metals which are to be protected, the corrosion inhibitors employed are complex, highly controlled mixtures containing a large number of ingredients. Inhibitors formulated for these systems as a rule contain one or more antioxidants in combination with alkaline ingredients.

A particularly effective corrosion inhibitor for organic fluid has been described in U.S. Patent 3,087,959, granted to me on Apr. 30, 1963, wherein the patented process is directed to the condensation reaction of 1,2-propylene glycol with sodium tetraborate decahydrate. This condensation reaction provided a considerably simplified and effective corrosion inhibiting additive in synthetic fluid media comprising glycols and ethers of glycols. While this previous process has been utilized to overcome the corrosive action of non-petroleum base hydraulic brake fluids and other synthetic type fluids, the condensate of said process was not sufficient without the contributory action of a phenolic or hydroquinone antioxidant. The prior art specification for inhibiting corrosion of the brake system metals, i.e., tin, steel, aluminum, cast iron, brass and copper was directed toward the combined usage of the alkaline type tetraborate condensation product with a suitable antioxidant, as mentioned above.

The inclusion of antioxidants increases the complexity of hydraulic brake fluids rendering such fluids more susceptible to interaction on prolonged storage or under various operating conditions. Antioxidants seldom exhibit complete compatibility with synthetic fluids, and they have deleterious effects on natural or synthetic rubber components in brake and cooling systems.

Further improvements in the tetraborate condensate are now possible in accordance with the present invention that achieves in a unified tetraborate composition the alkaline action and the antioxidant properties previously obtained by a combination of ingredients. The novel corrosion inhibitor of my present invention exhibits sufficient corrosion inhibiting properties to be effectively utilized as the sole inhibitor additive in synthetic fluids, such as the Ucons or other mixtures containing for example glycols, glycol-ethers, polyoxyglycols, castor oil and its derivatives, etc. Significantly, the present unified corrosion inhibitor not only has eliminated the need for phenolic and other antioxidants previously required for adequate protection of metals, but the present unified composition displays increased protection to various metals.

Therefore, it is an object of the present invention to provide a novel corrosion inhibitor which is capable of

**2**

increased anticorrosion protection to tin, steel, aluminum, cast iron, brass, copper or solder over other similar compositions used for this purpose.

Another object is to provide a novel tetraborate composition which is used effectively as the sole inhibitor in fluids composed of glycols, glycol ethers and including such other materials as polyoxyglycols or castor oil.

A further object is to provide a unified composition with enhanced properties for protecting metals greater than the properties of the separate constituents utilized in its synthesis.

A still further object resides in the process for forming a unified, stable composition which displays antioxidant properties and alkaline action.

Yet a further object provides for improved hydraulic and coolant fluids which include an improved tetraborate composition to inhibit their corrosive nature toward metals.

Other and further advantages of the present invention will become apparent from the following description and examples.

The corrosive inhibitor of this invention comprises the condensation product in which 1,2-propylene glycol is initially reacted with sodium tetraborate decahydrate, and then by proper control of such reaction, 2-butyne-1,4-diol is reacted with the tetraborate. The final condensation product combines both the propylene glycol and the acetylenic diol to the tetraborate. By proper control of the reaction, it is possible to restrict the initial condensation to one or two molecules of the glycol in order to involve the further condensation with the unsaturated molecule.

The unified composition of the invention is produced by adding the tetraborate in increments to the glycol at a temperature of  $85^{\circ}\text{C.} \pm 5^{\circ}\text{C.}$  It has been found essential to add the tetraborate incrementally and to allow each increment to dissolve before further addition. A single addition of the tetraborate does not lead to the condensation reaction but merely to a solution of borax in glycol. The total amount of tetraborate reacted with the glycol is about 20 to 30% by weight of the glycol. After this addition is completed, the temperature of the mixture is raised to  $105^{\circ}\text{C.}$ , and an amount of 2-butyne-1,4-diol equal to about  $\frac{1}{2}$  the weight of the borate is added to the mixture. Heating is continued until substantially all available water is evaporated from the reaction.

The resulting liquid formed by the present reaction is clear, viscous and amber in color. A significant theoretical consideration of the present unified composition is its increased ability to provide protection to metal surfaces by a two-fold attack on the surrounding fluid media. The present condensate (1) initially suppresses oxidation reactions in the surrounding fluid that lead to acid formation and (2) effectively neutralizes any acids which may appear after a prolonged period of operation. Thus, the present composition may be utilized as the sole corrosion inhibitor without the need for blending various ingredients to provide corrosion protection to metals.

The present process and compositions will now be explained in greater detail by means of the following preferred embodiments thereof.

**EXAMPLE I**

An amount of 1,2-propylene glycol weighing 700 grams was heated to a temperature of  $85^{\circ}\text{C.}$  with stirring. Powdered borax (sodium tetraborate decahydrate) weighing 210 grams and amounting to 30% by weight of the glycol was added to the liquid in three equal increments, allowing sufficient time after each addition for the powder to dissolve and form a clear mixture. After the third increment of borax was added, the mixture was heated to

105° C. and maintained at that temperature for one hour with stirring. At this point, 2-butyne-1,4-diol weighing 140 grams was added to the mixture, and the mixture was stirred at 105° C. for two additional hours. The resulting composition upon cooling was clear, amber and viscous.

The condensate which is a preferred embodiment of the invention is produced by reacting sodium tetraborate decahydrate with 2-butyne-1,4-diol in a ratio of 3:2, respectively. Effective ranges in which the constituents may be combined in accordance with the invention are expressed more conveniently in parts by weight:

| Constituent:                   | Parts by weight |
|--------------------------------|-----------------|
| 1,2-propylene glycol           | 1.00            |
| sodium tetraborate decahydrate | 0.2 to 0.3      |
| 2-butyne-1,4-diol              | 0.125 to 0.25   |

The inhibiting action of the present composition may be better explained by observing the effect of its molecular structures. In the initial reaction of 1,2-propylene glycol with sodium tetraborate decahydrate, the following series of condensates will be formed:



borate molecule has accepted only one (illustrated by I above) or possibly two (illustrated by II above) of the 1,2-propylene glycol molecules. If the sodium tetraborate molecule has accepted only one glycol molecule, the reaction with the 2-butyne-1,4-diol would then yield the following product:



Again, the reaction of 2-butyne-1,4-diol with the molecules of sodium tetraborate which have condensed with one or two 1,2-propylene glycol molecules can proceed as long as free —OH groups and B—O—B bonds are present. However, the condensation reaction depends on the length of time at which the reaction ingredients are heated together. It is unlikely that the reaction proceeds far enough to form compounds other than those represented in reactions IV and V above. The contention that further reactions are not involved in the present process is supported by the fact that when heating is continued, solids begin to form in the reaction. This is in agreement with the theoretical aspects that further condensation would result in solid materials. The present condensation product is prepared in a manner in which the glycol and diol are reacted separately at a temperature at which condensation proceeds rapidly and the water of the reaction is readily evaporated with a minimum loss of glycol.

#### EXAMPLE II

Sodium tetraborate decahydrate was added in several increments to 1,2-propylene glycol in a weight ratio of 1:5, respectively, while the mixture was being stirred and heated at 85° C. The addition was carried out at a rate which avoids accumulation of solids in the reaction mixture. Upon addition of the last amount of tetraborate,

This reaction can proceed as long as there are free —OH groups and B—O—B bonds. In the present process, however, the time allowed for the initial condensation with the 1,2-propylene glycol is carefully controlled to limit the extend of condensation per molecule. By the time the 2-butyne-1,4-diol is added, the sodium tetraborate

the temperature was raised to 105° C. and the mixture was stirred for one hour. An amount of 2-butyne-1,4-diol constituting  $\frac{2}{3}$  the weight of the sodium tetraborate decahydrate was added to the mixture at 105° C., and the mixture was continuously stirred and heated at 105° C. for an additional two hours. This temperature was found to be sufficient for evaporation of the water of the reaction with a concomitant minimal loss of glycol. Also, this temperature is low enough to reduce the possibility that volatile boron esters will form during the reaction.

The degree of condensation in this reaction may be determined by the method disclosed in copending application, Ser. No. 332,557, filed Nov. 8, 1963, which has issued as U.S. Patent 3,262,961 on July 26, 1966 to Charles B. Jordan, who is also the applicant herein, and wherein said method is based on a Karl Fischer reagent which is employed as a test solution to indicate the extent of water evaporated from the reaction. The reagent provides a convenient means for following the rate at which water is removed from the reaction and provides an accurate quantitative determination of the water content that remains in the condensation product. Normally, the heating step at 105° C. for two hours in an open vessel is sufficient to reduce the water content in the condensation product to a level of about 2.5%. Although, the water may be more desirably reduced to a level of about 1.5%, prolonged heating to achieve this degree of dryness may result in excessive condensation and formation of solids.

### EXAMPLE III

The condensation product in accordance with the invention may be prepared from a sodium tetraborate having various degrees of hydration. The procedure of the previous examples was repeated using sodium tetraborate pentahydrate (30% by weight of the glycol). The weight ratio of sodium tetraborate pentahydrate to 2-butyne-1,4-diol was 2:1, respectively. At the start, 5 moles of water were added to the glycol at 85° C. prior to the sodium tetraborate pentahydrate addition.

### EXAMPLE IV

A corrosion inhibitor in accordance with the invention may also be prepared using anhydrous sodium tetraborate. The addition of 10 moles of water to the glycol at 85° C. before the tetraborate addition enables the reaction mixture to remain fluid and readily stirrable throughout the reaction.

### EXAMPLE V

Condensation products in accordance with the reaction were also prepared by substituting ethylene glycol for the 1,2-propylene glycol in the process of Examples I and II. The tetraborate addition was on a 25% by weight based on the weight of ethylene glycol, and the diol addition was on an 18% by weight based on the weight of ethylene glycol. The product remained fluid throughout the reaction.

#### Test No. 1

Corrosiveness of brake fluids is determined by testing metal strips of the six metals (tin, steel, aluminum, cast iron, brass and copper). The test specified in Military Specification MIL-H-13910a involves clean strips of metal immersed in a brake fluid containing 3% of the present corrosion inhibitor by weight. The strips are kept in the fluid for 120 hours at a temperature of 210°  $\pm$  3° F. Following this test period, the strips are then visually examined for evidence of corrosion, pitting, etching and discoloration. The strips are then weighed to the nearest 0.1 milligram and the weight loss per unit area of each strip is calculated. In order to pass the test satisfactorily, no pitting or etching should occur and very little discoloration of the strips is permitted if the fluid is to be accepted for government use. The brake fluid in accordance with the aforementioned Military Specification which is used

to compare the effectiveness of corrosion inhibitors consists of the following composition:

| Constituent:                       | Percent by weight |
|------------------------------------|-------------------|
| Butoxy polypropylene glycol        | 22.0              |
| Diethylene glycol monomethyl ether | 35.0              |
| Ethylene glycol monobutyl ether    | 20.0              |
| Ethylene glycol monoethyl ether    | 20.0              |
| Corrosion inhibitor                | 3.0               |

10 The present corrosion inhibitor composition which was tested in the above brake fluid was prepared by reacting the following constituents in accordance with the present process:

| Constituent:                   | Parts by weight |
|--------------------------------|-----------------|
| 1,2-propylene glycol           | 1.00            |
| Sodium tetraborate decahydrate | .30             |
| 2-butyne-1,4-diol              | .20             |

15 The prior art inhibitor disclosed in U.S. Patent 3,087,959 was formed by reacting 1,2-propylene glycol with sodium tetraborate decahydrate. This condensate was tested in the brake fluid shown above as a comparison with the present inhibitor. In accordance with the previous requirement, an antioxidant compound was combined with the condensate. Di-tertiarybutyl paracresol was mixed with the condensate in about 66% condensate and 34% antioxidant, a ratio in which these materials have been previously combined as an oxidation inhibitor.

20 25 30 The results of the test are given in the table below:

TABLE I

| Metal     | Present Inhibitor  |                                            | Prior Art Inhibitor |                                            |
|-----------|--------------------|--------------------------------------------|---------------------|--------------------------------------------|
|           | Visual Inspection  | Weight Loss (Milligrams/cm. <sup>2</sup> ) | Visual Inspection   | Weight Loss (Milligrams/cm. <sup>2</sup> ) |
| Tin       | No change          | .00                                        | No change           | .00                                        |
| Steel     | do                 | .00                                        | do                  | .01                                        |
| Aluminum  | do                 | .00                                        | do                  | .01                                        |
| Cast iron | do                 | .00                                        | do                  | .00                                        |
| Brass     | Very slight stains | .02                                        | Heavy stains        | .06                                        |
| Copper    | Slight stains      | .04                                        | do                  | .11                                        |

35 55 There was no pitting or etching, nor were there any deposits on the strips. The present corrosion inhibitor showed marked improvement with brass and copper. Weight losses with the brass and copper metals were about three times higher with the prior art inhibitor.

60 The present inhibitor has been found effective when employed as an additive in the range of 2.5-6% by weight.

#### Test No. 2

65 In order to compare the improvement by the present unified corrosion inhibitor over a similar composition containing the same constituents but in separate form, the following test was devised:

70 The prior art condensate, employed in the previous test, was mixed with an equivalent amount of 2-butyne-1,4-diol to test the efficacy of the combination as a corrosion inhibiting composition. The procedure of the previous test was employed, and the results obtained by this combination of ingredients are now compared with the test results obtained with the present inhibitor.

TABLE II

| Metal          | Condensate+Diol      |                                            | Present Inhibitor         |                                            |
|----------------|----------------------|--------------------------------------------|---------------------------|--------------------------------------------|
|                | Visual Inspection    | Weight Loss (Milligrams/cm. <sup>2</sup> ) | Inspection                | Weight Loss (Milligrams/cm. <sup>2</sup> ) |
| Tin-----       | No change-----       | .00                                        | No change-----            | .00                                        |
| Steel-----     | do-----              | .00                                        | do-----                   | .00                                        |
| Aluminum-----  | do-----              | .00                                        | do-----                   | .00                                        |
| Cast iron----- | do-----              | .00                                        | do-----                   | .00                                        |
| Brass-----     | Heavy staining-----  | .06                                        | Very slight staining----- | .02                                        |
| Copper-----    | Slight staining----- | .05                                        | Slight staining-----      | .04                                        |

The above test indicates that the mere presence of the acetylenic compound does not provide the improvement which is achieved by combining the ingredients into a single inhibitor composition.

#### Test No. 3

The stability of the present inhibitor in the brake fluid was also tested. Strips of aluminum and cast iron, spaced .001 inch were inserted in the fluid and 2% benzoyl peroxide by weight was added. The fluid was then heated at 158° F. for 168 hours. The test revealed no weight loss to either the aluminum or cast iron strip.

Antifreeze compounds are composed of diluted and undiluted glycols, alcohols and glycol-ethers. The present inhibitor was tested in an antifreeze solution made up of 50% glycol and 50% water by including it therein in 3% by volume. The corrosiveness of the solution was then tested by metal strips (solder, steel, aluminum, cast iron, brass and copper) which were immersed in the antifreeze solution at 180° F. for a period of 192 hours, during which time the antifreeze solution was aerated and refluxed. After 192 hours the metal strips were removed from the solution, inspected and weighed. The results from this test are compared in Table III with the performance of a standard antifreeze solution containing borax as the corrosion inhibitor.

TABLE III

| Metal          | Present Inhibitor—Visual Inspection | Standard Inhibitor—Visual Inspection |
|----------------|-------------------------------------|--------------------------------------|
| Aluminum-----  | Slightly stained-----               | Heavily stained-----                 |
| Copper-----    | No change-----                      | Moderately stained-----              |
| Solder-----    | do-----                             | Slightly etched and pitted-----      |
| Brass-----     | do-----                             | Heavily stained-----                 |
| Steel-----     | do-----                             | Slightly stained-----                |
| Cast iron----- | Very slightly stained-----          | Do-----                              |

The present inhibitor decreases corrosive action on all coolant system metals. It is especially beneficial to aluminum on which a protective oxide coating is readily formed which acts as a shield against corrosion and erosive action. The present unified inhibiting composition is also compatible with all present day antifreeze additives, such as mercaptobenzylthiazole and its salts, and they have no deleterious effects on the rubber components.

The present corrosion inhibitor is miscible in all proportions with water. This is particularly desirable for organic coolants whether they are diluted or undiluted. The inhibitor may also continue to protect brake systems in which a large amount of water has accumulated.

The present condensate is substantially stable under prolonged storage and is not affected by a raise in temperature. Any oxidation or decomposition of the organic constituents will be neutralized by the reserve alkalinity of the condensate. The stability of the triple bond excludes attack by oxygen from the air, but permits attack of oxidations occurring in the liquid.

Thus it is apparent from the present specification that the novel condensate of the present invention exhibits

superior inhibiting properties against corrosion. It is also capable of being utilized more effectively as the sole inhibitor in organic fluids thus allowing for greater stability and uniformity than the previous mixtures which were used for this purpose.

The invention is not limited to the specific examples and embodiments herein disclosed, but includes all such modifications and adaptations thereof made within the spirit of the invention as set forth in the appended claims.

Having particularly described this invention, that which is claimed is:

1. The process of preparing a corrosion inhibiting composition which comprises:

adding powdered sodium tetraborate decahydrate to 1,2-propylene glycol at 85° C. in increments in a total amount of about 20 to 30 percent by weight of said glycol to form a solution,

heating said solution at about 105° C. for about 1 hour, adding 2-butyne-1,4-diol to said solution in an amount of about 12.5 to 25 percent by weight of said glycol, and

heating the resulting solution at about 105° C. to evaporate the water of the reaction to a level of about 1.5-2.5 percent by weight of said solution.

2. The process of preparing a corrosion inhibiting composition in accordance with claim 1 in which the resulting solution is heated at 105° C. for a period of two hours.

3. A corrosion inhibiting composition prepared by the process of claim 1.

4. The process as set forth in claim 1 wherein the sodium tetraborate decahydrate is added in about 30 percent by weight of said glycol and said 2-butyne-1,4-diol is added in about 20 percent by weight of said glycol.

5. A corrosion inhibiting composition prepared by the process of claim 4.

6. A corrosion inhibiting composition prepared by the process of claim 1 wherein said 2-butyne-1,4-diol is added in an amount equal to about  $\frac{2}{3}$  the weight of said tetraborate.

7. The process of preparing a corrosion inhibiting composition which comprises:

adding to 1,2-propylene glycol an amount of water corresponding to  $(10-n)$  times the molar equivalent of sodium tetraborate to be added in said process, where  $n$  represents the molar ratio of the water of hydration associated with said sodium tetraborate and is a number less than 10 and which may be zero,

heating said 1,2-propylene glycol and water to 85° C. adding in increments said sodium tetraborate in a state of hydration corresponding to the formula



in a total amount of about 20 to 30 percent by weight of said glycol times the ratio of the molecular weight of  $\text{Na}_2\text{B}_4\text{O}_7 \cdot n\text{H}_2\text{O}$  to  $\text{Na}_2\text{B}_4\text{O}_7 \cdot 10\text{H}_2\text{O}$  to form a solution,

heating said solution to 105° C. for about 1 hour, adding 2-butyne-1,4-diol in an amount of about 12.5 to 25 percent by weight of said glycol, and

heating the resulting solution at about 105° C. to evaporate the water of the reaction to a level of about 1.5-2.5 percent by weight of said solution.

#### References Cited

##### UNITED STATES PATENTS

- 2,979,524 4/1961 Wright et al. 252—75  
 2,982,733 5/1961 Wright et al. 252—75  
 3,087,959 4/1963 Jordan 260—462

70 LEON D. ROSDOL, Primary Examiner.

SAMUEL H. BLECH, Examiner.

S. D. SCHWARTZ, Assistant Examiner.